

## UNITED STATES PATENT OFFICE

FRANCIS GÁBOR AND PAUL KLEIN, OF BUDAPEST, HUNGARY, AND ANDREW SZEGVÁRI, OF AKRON, OHIO, ASSIGNEES, BY MESNE ASSIGNMENTS, TO AMERICAN ANODE, INC., A CORPORATION OF DELAWARE

PROCESS FOR THE PRODUCTION OF HOMOGENEOUS RUBBER DEPOSITS FROM RUBBER LATEX

No Drawing. Application filed July 22, 1926, Serial No. 124,285, and in Germany September 4, 1925.

In specification of the Patent No. 1,548,689 we have stated that in the production of rubber deposits by electrophoretic means electrolysis of the electrolytes contained in the dispersion liquid of the rubber latex takes place simultaneously with the deposition of the rubber, gas being developed at the anode and we have further stated that it is owing to this anodic generation of gas that homogeneous rubber deposits cannot be obtained in this manner. This recognition led to the proposal made in the specification of the aforesaid patent, to enable the gases set free at the anode to escape by specially separating the point of production of the anodic gases from the point of formation of the rubber deposit. This spacial separation was effected by means of a porous base which was interposed as depositing base, between the anode and the cathode. In the specification of our application No. 35,246, filed June 5, 1925, we specified further means for enabling homogeneous precipitates to be obtained or for obviating the detrimental influence of the electrolytic separation of gas at the anode, which consisted in suppressing the liberation of gases. This was effected by employing in the electrophoretic device substances adapted to prevent the liberation of gases and more particularly by employing anodes which contain substances or are composed of substances adapted to combine the anodic gases in any suitable manner in order to enable homogeneous rubber precipitates to be produced also immediately upon the surface of electrically conductive anodes.

We have found that all metallic anodes, even for example lead or zinc anodes which it might be assumed would enter into chemical combination with the gases liberated thereupon by electrolysis and would consequently by combining with these gases, especially the oxygen, prevent the liberation of gas, offer difficulties in preventing the development of gas on the anode and in producing from latex preserved in the usual commercial way, completely homogeneous precipitates.

We have now ascertained that when employing metallic deposition bases, it is not sufficient merely to select a suitable metal

for the anode but that the prevention of the development of gases at the anode with certainty, in order to produce homogeneous caoutchouc deposits also depends on the quality of the corresponding preliminary treatment of the commercial latex. We have especially found that commercial preserved latex contains substances, in the presence of which the formation of gases at the anode under the influence of the electric current is favourably influenced and that these substances must be removed from the latex to be electrophoretically treated for the production of rubber goods, or must be reduced to harmless proportion. The removal or decrease of the detrimental substances can for example be effected by the partial or entire removal or by partial or entire transformation of same into a harmless form.

Commercial preserved latex contains for example 0.5-1% ammonia. We have found that the greater part of this ammonia must be removed. Experiments have shown that when treating latex containing 33% rubber and employing anodes of zinc, cadmium, lead and similar metals or alloys thereof it is advantageous to reduce the ammonia content of the latex (33% rubber content) to a total alkalinity of about 0.09 normal ammonium hydroxide solution or below. On the other hand however it has been found that for the quality of the homogeneous rubber deposit obtained and for the behaviour of the latex, it is advantageous not to remove the ammonia content entirely. The upper limit and the most advantageous proportion of the ammonia content depend on the condition and the concentration of the latex employed, the temperature, the substance of the anode and on other circumstances, and must always be ascertained by experiments.

The decrease or removal of the preventing agents can be effected by dialysis or by washing out the latex, for example by concentrating same by centrifuging and subsequent dilution. Such operations may also effect the removal or decrease of other constituents of the latex which might also favour the development of gases at the anode or might for other reasons, otherwise detrimentally influ-

55

60

65

70

75

80

85

90

95

100

ence the process or the quality of the product.

If the substance to be removed is volatile, as is the case for example with the ammonia at present generally employed, the amount thereof may also be diminished by evaporation, aeration, or by heating or by employing these measures simultaneously. Experiments have shown that the ammonia content can be reduced to the required small amount, for example by heating the latex to about 70° C. for some hours without endangering the same.

Another method of eliminating or diminishing or removing the preserving agent consists in transforming the same into a compound which does not tend to form gas or any otherwise detrimental compound during the electrophoretic deposition of the rubber. Thus for example the ammonia content of the commercial preserved latex can be counteracted by formaldehyde or its polymers, in which case the ammonia is transformed into hexamethylentetramine and hydroxyl ion concentration is correspondingly reduced. Other carbonyl-containing CO compounds can be employed in the same way.

Another method of transforming the detrimental substances in case they should be alkaline, consists in merely neutralizing them, in which case however limits are set to the addition of strongly acid substances, by the danger of coagulation. Nevertheless the acid required for the neutralization can frequently be produced in the latex itself (for instance by the oxidation of aldehyde).

Another possibility of avoiding the formation of gas consists in employing for preserving latex, instead of ammonia, other alkaline acting substances which do not incline to the formation of gases at all during the electrophoretic deposition of the rubber or which may be employed only in such small amounts that they do not produce any formation of gas during the electrophoretic deposition.

Instead of alkaline additions, substances having a strongly germicidal action such as for example thymol or the hydrocupreine compounds known as Eucupinotoxine and vucine may be employed for preserving the latex in which case such small amounts are sufficient that they do not come into consideration for the electrolytic gas-formation.

Even if the ammonia preserved latex has been freed of its ammonia-content to the lowest admissible extent prior to treatment, it is generally preferable to add to the latex a disinfectant which does not produce any detrimental gas formation.

With latices prepared in the above described manner perfect completely homogeneous rubber deposits can be obtained directly on zinc, cadmium, iron and lead anodes as well as upon anodes which consist of certain alloys containing the above metals

(for example an alloy containing 90% zinc and 10% antimony).

The experiments hitherto made appear to indicate, although this has not been definitely ascertained, that the above described behaviour of the latex depends on the circumstance that on the one hand electrodes have to be employed which, in the course of the electrophoretic deposition of the rubber under the given conditions or in the presence of the electrolytes employed are continuously ionized, being for example dissolved by the oxidation products produced by the electrolysis of the metal of the anode and that on the other hand the concentration of the electrolyte supplying the hydroxyl ion in relation to the rate of dissolution of the anode or of the oxidation products formed from the anode metal is reduced to such an extent that it is merely sufficient for secondary reactions and the hydroxyl ions are unable to effect a primary discharge which would lead to the formation of gases.

The decrease in concentration of the gas-forming electrolyte by diluting the latex does not lead to the result because commercial preserved latex had to be diluted to a six or seven fold extent for this purpose and it is impossible to produce from such a diluted latex suitable rubber deposits since the same do not exhibit a smooth surface, and moreover the speed of deposition of the rubber is considerably decreased.

We have also found that even in the presence of substances inducing gas formation for example of the ammonia contained in commercial preserved latex, it is possible to suppress the formation of gases if the electrophoresis is commenced at a current density at which the jump in potential at the anode is insufficient to effect electrolysis with its attendant gas formation that is to say below about 1.7 volts. As the electrophoretic deposition of the rubber progresses the electrical resistance may be increased. In this case the voltage can be gradually increased without increasing the jump in potential at the anode. In this process however the formation of the deposit proceeds extremely slowly and the thickness of the non-porous layer appears to be very greatly limited.

The condition of the rubber deposit formed directly on the surface of the metal anode can be influenced in an undesirable manner by the too immediate influence of the metal entering into solution from the anode for which reason it may be advantageous to provide the anode with a liquid absorbing non-metallic protection as for example a thin coating of tanned or untanned gelatine, collodion, and the like which is adapted to prevent the direct contact of the rubber with the metal. This liquid-absorbing coating which is however impermeable to gas bubbles must be saturated prior to dipping the

anode into the latex, with any suitable medium adapted favourably to influence the coagulation of the rubber in the given arrangement. The surface of the anodes may be smoothed or may be provided with any desired raised or sunk pattern. The individual parts of the anodic surface may consist of metals upon which formation of gas occurs and upon which a correspondingly porous deposit is accordingly produced. Portions of the anode on which no deposit is desired may be provided with an electrically insulating coating.

Moreover individual portions of the deposition base may consist of porous substances permeable to liquid and arranged in front of the anode in the manner described in the specification of Patent No. 1,548,689 whilst at the remaining portions of the deposition base, the deposit is formed directly upon the surface of the anode.

In other respects the deposition when using metallic deposition bases offers similar possibilities to those described in the specification of Patent No. 1,548,689 in connection with the deposition upon porous non-conducting bases i. e. various additional substances for example vulcanizing agents, vulcanizing accelerators, filling materials, colouring matters and the like may be mixed with the latex, the deposit may be produced upon moulds entirely immersed in the latex or upon endless bases (drums or bands) passing through the latex in a continuous manner and in both cases fibrous materials or fabric insertions can be employed or saturated with rubber.

When employing metallic moulds the rubber deposit can be dried and vulcanized upon the moulds themselves or the deposit obtained can be removed from the moulds prior to vulcanization, since the deposits produced by means of the above-described process possess sufficient strength and elasticity for this purpose.

It should be remarked that the expression "rubber latex" is intended to denote vulcanized or unvulcanized latex both free from filling materials as well as containing filling materials, vulcanizing agents, vulcanizing accelerators, colouring matters and other additional substances.

It should be well understood that the above described electrophoretic deposition process can be advantageously carried out with the auxiliary means described in the specifications of our co-pending applications Nos. 35,199 and 35,246, filed June 5, 1925.

Having now particularly described and ascertained the nature of our said invention and in what manner same is to be performed, we declare that what we claim is:—

1. The process of making by electric means homogeneous rubber deposits from commercial rubber latex which comprises eliminat-

ing to a substantial extent in the commercial rubber latex substances tending to liberate gases at the deposition base, immersing in the treated latex a deposition base comprising a metal or alloy substantially incapable under the influence of a rubber depositing electric current of forming gases thereon in the treated latex, and passing through said latex and deposition base an electric current capable of electrophoretically depositing rubber from said latex at said base.

2. The process set forth in claim 1 in which the deposition base is composed of metals capable of continuously ionizing during the electrophoretic deposition.

3. The process set forth in claim 1 in which the deposition base comprises a metal of a class including zinc, cadmium, iron, lead and alloys of these metals.

4. The process of making homogeneous rubber deposits from commercial rubber latex by electrophoretic deposition which comprises eliminating to a substantial extent in the commercial rubber latex substances tending to liberate gases at the deposition base and adding to the treated latex preserving agents substantially incapable of liberating gas at the deposition base during electrophoretic deposition, immersing in the treated latex a deposition base comprising a metal or alloy substantially incapable under the influence of a rubber depositing electric current of forming gases thereon in the treated latex, and passing through such treated latex and deposition base an electric current capable of electrophoretically depositing rubber from said latex at said base.

5. The process as set forth in claim 4 in which the preserving agents comprise a substance of a class capable of retarding bacterial action in the latex.

6. The process of making homogeneous rubber deposits from ammonia-preserved latex by electrophoretic deposition which comprises reducing the ammonia concentration in the latex to such an extent that substantially no gas formation takes place at the deposition base during electrophoretic deposition, immersing in the treated latex a deposition base comprising a metal substantially incapable under the influence of an electrophoretic depositing current of forming gases thereon and passing through such treated latex and deposition base an electric current capable of electrophoretically depositing rubber from said latex at said base.

7. The process of making homogeneous rubber deposits from ammonia-preserved latex by electrophoretic deposition which comprises reducing the ammonia content in the latex to a 0.1 normal solution or below, immersing in the treated latex a deposition base comprising a metal substantially incapable under the influence of an electrophoretic depositing current of forming gases there-

- on and passing through such treated latex and deposition base an electric current capable of electrophoretically depositing rubber from said latex at said base.
5. 8. The process of making homogeneous rubber deposits from ammonia-preserved latex by electrophoretic deposition which comprises reducing the ammonia content of the latex by adding to the latex a substance reacting with the ammonia, immersing in the treated latex a deposition base comprising a metal substantially incapable under the influence of an electrophoretic depositing current of forming gases thereon and 10 passing through such treated latex and deposition base an electric current capable of electrophoretically depositing rubber from said latex at said base.
9. The process of making homogeneous rubber deposits from ammonia-preserved latex by electrophoretic deposition which comprises reducing the ammonia content of the latex by adding thereto substances capable of reducing the alkalinity thereof, immersing in the treated latex a deposition base comprising a metal substantially incapable under the influence of an electrophoretic depositing current of forming gases thereon and 15 passing through such treated latex and deposition base an electric current capable of electrophoretically depositing rubber from said latex at said base.
10. The process of making homogeneous rubber deposits from ammonia-preserved latex by electrophoretic deposition which comprises reducing the ammonia content of the latex by adding an aldehyde thereto, immersing in the treated latex a deposition base comprising a metal substantially incapable 20 under the influence of an electrophoretic depositing current of forming gases thereon and passing through such treated latex and deposition base an electric current capable of electrophoretically depositing rubber from said latex at said base.
11. The process of making homogeneous rubber deposits from ammonia-preserved latex by electrophoretic deposition which comprises reducing the ammonia content of the latex by adding formaldehyde thereto, immersing in the treated latex a deposition base comprising a metal substantially incapable under the influence of an electrophoretic depositing current of forming gases thereon and 25 passing through such treated latex and deposition base an electric current capable of electrophoretically depositing rubber from said latex at said base.
12. The process of making homogeneous rubber deposits from preserved rubber latex which comprises reducing the total alkalinity of the latex to a 0.1 normal solution or below, bringing a deposition base in contact with the treated latex, and depositing a layer of rubber 30 from the latex on the deposition base.
13. The process of making homogeneous rubber deposits from preserved rubber latex which comprises adding to the latex a substance capable of reducing the alkalinity of the latex, bringing a deposition base in contact with the treated latex, and depositing a layer of rubber from the latex on the deposition base.
14. The process of making homogeneous rubber deposits from preserved rubber latex which comprises adding an aldehyde to the latex, bringing a deposition base in contact with the treated latex, and depositing a layer of rubber from the latex on the deposition base.
15. The process of making homogeneous rubber deposits from preserved rubber latex which comprises adding formaldehyde to the latex, bringing a deposition base in contact with the treated latex, and depositing a layer of rubber from the latex on the deposition base.
16. The process of making homogeneous rubber deposits from latex preserved with ammonia or amines which comprises reducing the total alkalinity of the latex by addition of substances reacting with the ammonia or amine, bringing a deposition base in contact with the treated latex, and depositing a layer of rubber from the latex on the deposition base.
17. The process of making homogeneous rubber deposits from latex preserved with ammonia or amines which comprises adding an aldehyde to the latex, bringing a deposition base in contact with the treated latex, and depositing a layer of rubber from the latex on the deposition base.
18. The process of making homogeneous rubber deposits from latex preserved with ammonia or amines which comprises adding formaldehyde to the latex, bringing a deposition base in contact with the treated latex, and depositing a layer of rubber from the latex on the deposition base.
- In testimony whereof we affix our signatures.
- FRANCIS GÁBOR.  
PAUL KLEIN.  
ANDREW SZEGVÁRI.